

J. A. SINGMASTER, F. G. BREYER AND E. H. BUNCE.

## MANUFACTURE OF ZINC OXID.

APPLICATION FILED JULY 22, 1919.

1,322,142.

Patented Nov. 18, 1919.

3 SHEETS—SHEET 1.



J. A. SINGMASTER, F. G. BREYER AND E. H. BUNCE.

## MANUFACTURE OF ZINC OXID.

APPLICATION FILED JULY 22, 1919.

1,322,142.

Patented Nov. 18, 1919.

3 SHEETS—SHEET 2.



## INVENTORS

INVENTORS  
Frank G. Breyer  
James A. Singmaster  
BY Carl H. Bance  
Bernie, Danis, Marnen, + Edmund

## ATTORNEYS

J. A. SINGMASTER, F. G. BREYER AND E. H. BUNCE.  
MANUFACTURE OF ZINC OXID.  
APPLICATION FILED JULY 22, 1919.

1,322,142.

Patented Nov. 18, 1919

3 SHEETS—SHEET 3.



INVENTORS  
Frank G. Breyer,  
James A. Singewarter  
BY Carl H. B. Once  
Genie, Davis, Marin, Edwards

ATTORNEYS

# UNITED STATES PATENT OFFICE.

JAMES A. SINGMASTER, OF NEW YORK, N. Y., AND FRANK G. BREYER AND EARL H. BUNCE, OF PALMERTON, PENNSYLVANIA, ASSIGNEES TO THE NEW JERSEY ZINC COMPANY, OF NEW YORK, N. Y., A CORPORATION OF NEW JERSEY.

## MANUFACTURE OF ZINC OXID.

1,322,142.

Specification of Letters Patent. Patented Nov. 18, 1919.

Application filed July 22, 1919. Serial No. 312,567

To all whom it may concern:

Be it known that we, JAMES A. SINGMASTER, residing at New York city, county and State of New York, FRANK G. BREYER and EARL H. BUNCE, both residing at Palmerton, county of Carbon, State of Pennsylvania, have invented certain new and useful Improvements in the Manufacture of Zinc Oxid, (Case E;) and we do hereby declare the following to be a full, clear and exact description of the invention, such as will enable others skilled in the art to which it appertains to make and use the same.

This invention relates to the production of zinc oxid or leaded zinc oxid by the Wetherill process, and has for its objects the provision of an improved method of producing zinc oxid, or leaded zinc oxid, by the Wetherill process, in a continuous operation.

Zinc oxid and leaded zinc oxid are principally produced in commercial practice by the so-called Wetherill process. By the expression "Wetherill process", as we have used the same herein, is to be understood the furnacing step of the process for producing zinc oxid, or leaded zinc oxid, as a finished commercial product, or as a zinc oxid (or zinc-lead) concentrate, or in any other form, in which a charge of the zinkiferous (or zinkiferous and plumbiferous) material mixed with a reducing agent and spread on an ignited bed of fuel is subjected to a combustion supporting blast or draft and brought to a sufficiently high temperature to reduce the compounds of zinc and volatilize the reduced metal (and to reduce and (or) volatilize the compounds of lead when present) without bringing the charge to a condition where it becomes impervious to the blast or draft; the entire charge being supported on a furnace hearth or grate designed to hold it without letting any considerable part drop through, and the worked-off material being discharged as a clinker or sinter. The "furnacing step" is independent of the subsequent treatment of the laden furnace gases and of the collection of the zinc oxid or leaded zinc oxid.

In the commercial production of zinc oxid (including leaded zinc oxid) by means of the Wetherill process, it has heretofore been customary to first charge upon the perfo-

rated hearth or grate of the present day type of zinc oxid furnace a layer of "buckwheat" 55 anthracite coal (which is thereupon ignited by the residual heat of the furnace) and by means of a forced draft or blast of air to bring this initial layer of coal to well-developed combustion. Upon this layer of "bed 60 coal" is then charged the customary mixture or "working charge" characteristic of the Wetherill process, that is to say, a mixture of finely-divided reducing coal with the finely-divided zinkiferous (or zinkiferous 65 and plumbiferous) material, such as zinc silicate, roasted zinc blendes, roasted so-called "mixed sulfids" of zinc and lead, spelter-retort residues, or other reducible zinc-containing (or zinc and lead containing) material at the disposal of the operator. The forced air draft is continued, and, when the familiar flames of greenish tint, known as "zinc candles", begin to make their appearance above the upper surface of the 75 charge, indicating that the reduction and volatilization of the zinc and its oxidation to the form of fume is well under way, the products of combustion carrying the zinc oxid fume and other volatilized metallic compounds are conveyed through the customary cooling flues, etc., to the bag-room wherein, in a cooled condition, they filter through the bags and pass off into the atmosphere, leaving the fume collected in the interior of 80 the bags, from which it is removed at convenient intervals. The furnace operation is continued until the production of fume therefrom in appreciable quantity ceases, whereupon the residual charge, which is, to 85 a large extent, sintered together, is broken up by long-handled rabbles and pried up and lifted or scraped out through the furnace doors into a receiving pit, or the like, preparatory to the starting of a new operation. The coal or other carbonaceous material of the charge serves the two-fold purpose of furnishing a reducing agent for effecting the reduction of the zinkiferous, or zinkiferous and plumbiferous, material of 90 100 the charge and of furnishing, by combustion, the necessary degree of heat to bring these materials to the reducing temperature characteristic of the process.

As thus ordinarily practised, the above 105 described furnace operation is attended with

certain defects interfering with its full efficiency. Prominent among these defects is the inevitable tendency to the formation of blow-holes or craters at various regions of the charge. These blow-holes represent severally the paths of least resistance for the blast in its passage through the charge and to the extent to which they develop in the progress of the operation they interfere with the uniform distribution of the air in its upward passage and produce "hot spots" representing excessive temperatures as compared with other regions of the charge. From time to time, the workmen endeavor to eliminate these blow holes or hot spots, as far as is feasible, by rabbling the upper surface of the charge, thereby filling in the blow holes or breaking up their continuity; but in spite of the palliative effect of these expedients (which, moreover, consume considerable of the workman's time and attention), it is impossible to obtain uniform working conditions throughout the entire extent of the charge; so that there is not only waste of fuel, and the production locally of higher temperatures than is desirable, but the residues taken from the furnace at the termination of the operation contain notable percentages of zinc. The zinc contained in these residues cannot ordinarily be recovered commercially, and, when the residues are employed in the manufacture of spiegeleisen or for the recovery of their lead or other values, the presence of the residual zinc is objectionable, for the reason that, when volatilized and oxidized in the furnace, it interferes to a greater or less extent with the normal furnace operation and tends to collect in and obstruct the furnace flues.

A further defect of the above described furnace practice is that the forced draft, which is employed under relatively considerable pressure, tends to project into the free space above the charge more or less dust, particularly in the region of the blow-holes referred to, and this dusting is further aggravated by the rabbling operations; consequently, in addition to the metallic fume, the products of combustion carry with them from the furnace a notable proportion of dust in the form of fine particles of unreduced ore, carbon, ash, and the like, which tend to contaminate the fume proper and damage its color and marketability.

There are, furthermore, certain requirements of the practice of the Wetherill process as heretofore conducted which hamper the operator in the selection of the quality and size both of the coal and of the zinkiferous material employed in making up the charge. Thus, the requirement that the charge shall be sufficiently permeable for the passage of the air necessitates the use of a mixture of coal and zinkiferous material of a fairly coarse grade. Serious difficulties

are encountered in the use of the small sizes of buckwheat coal, and only a fractional part of the zinkiferous constituents of the charge can consist of such extremely finely-divided materials as flotation concentrates, zinc precipitates, flue-dust containing zinc, or the like.

The aforementioned defects and difficulties of the heretofore customary commercial practice of the Wetherill process may be overcome to a very remarkable extent by modifying this practice in accordance with the improvements described in the application for Letters Patent of the United States of Frank G. Breyer, James A. Singmaster and Albert E. Hall, Serial No. 270,179, filed January 8, 1919. These improvements consist in supplying either or both the bed fuel and the working charge to the furnace hearth in the form of briquets. The improved results attendant upon this modification in the prior customary practice of the Wetherill process are described in detail in the aforementioned application.

In commercial practice, the furnace in which the Wetherill process is carried out has heretofore been generally constructed as a block containing several grate units. Thus, it is customary to build the furnace or block with four to twelve grate units, each of which may, for example, be about four feet wide and about ten feet long. These grate units may be arranged side by side, or half of the units may be arranged side by side and the two halves arranged back to back. The purpose of this arrangement is to get relative continuity of action in the treatment of charges that individually are worked intermittently. Thus, while the operation of the furnace or block may, for practical purposes, be considered more or less continuous, the operation with respect to any individual grate unit is intermittent.

One of us, James A. Singmaster, has described and claimed in U. S. Letters Patent Nos. 1,112,853 and 1,112,854, patented Oct. 6, 1914, a process and apparatus for producing zinc oxid by the Wetherill process in which the ignited charge is advanced through a suitable combustion zone in a continuous manner. One of the difficulties encountered in attempting to advance through a combustion zone a charge of finely-divided materials, such as the heretofore customary Wetherill process charge, supported on a movable perforated grate, is that of providing a seal at the sides of the charge. The relative motion between the side walls of the combustion zone and the moving charge provides a very susceptible region for the air blast to break through the charge, and because of this relative movement it is practically impossible to provide an effective seal between the moving charge and the stationary furnace walls with which it directly

contacts. In the aforementioned Letters Patent this difficulty is avoided by supporting the charge, during its movement through the combustion zone, on grate sections so arranged that the moving charge is not in contact with any stationary element, the grate sections themselves being designed to effect the desired seal between the movable and stationary parts.

10 We have now discovered that very remarkable results are attained, when the Wetherill process is carried out as a continuous operation by advancing an ignited working charge through a suitable combustion zone, by supplying to the moving furnace hearth either or both the layer of bed fuel and the working charge in the form of briquets. The present invention thus contemplates advancing through a suitable combustion zone a 15 working charge containing a briquetted mixture of zinkiferous, or plumbiferous-zinkiferous, material and a reducing agent spread on an ignited layer of bed fuel, also preferably in the form of briquets, and simultaneously passing a combustion supporting 20 gas into the charge.

In our preferred practice, the working charge, in the form of briquets made up of a mixture of zinkiferous material, or plumbiferous-zinkiferous material, and an appropriate reducing agent, is spread upon a well ignited layer of bed fuel also in the form of briquets, and the entire charge supported on a perforated furnace hearth, is advanced 25 through a suitable combustion zone or chamber. The fuel briquets may, if desired, contain such a percentage of the zinkiferous or plumbiferous-zinkiferous material as will not interfere with their normal function.

30 The bed fuel briquets may be prepared by compressing finely divided coal, together with a suitable binder, such, for example, as the concentrated waste sulfite liquor of the sulfite paper pulp industry. Various forms 35 and grades of carbonaceous material are available for the bed fuel briquets. Thus, for example, anthracite coal below the No. 3 buckwheat size, such as No. 4 buckwheat, colliery washings, "dirt" coal, "dust" coal, 40 as well as coke breeze, may be utilized in the production of the bed fuel briquets. The bed fuel briquets are of such size and shape as to materially reduce the resistance to the combustion supporting gas, and nevertheless 45 to supply such a substantially uniform substratum for the support of the superposed working charge as to give free access therethrough and practically equal distribution thereto of the combustion supporting gas.

50 To this end, the bed fuel briquets, as well as the working charge briquets, should be of substantially uniform size, and preferably of such shape that they roll or tumble easily over one another. Thus, we have found the 55 so-called pillow block, eglette, rounded pil-

low block, over-stuffed pillow, and similar shapes well suited to the purposes of the invention.

While the working charge consisting of a mixture of zinkiferous, or zinkiferous and plumbiferous, material and an appropriate reducing agent may be supplied to the ignited layer of bed fuel briquets in an unbriqueted form, we prefer to briquet the working charge because of the many attendant advantages. Furthermore, we wish it to be understood that the zinkiferous, or zinkiferous and plumbiferous, material may be briqueted alone, without briquetting the reducing agent, or the reducing agent may be 70 briqueted alone without briquetting the zinkiferous, or zinkiferous and plumbiferous, material, or the reducing agent and the zinkiferous, or zinkiferous and plumbiferous, material may be separately briqueted. However, our preferred practice is to briquet a 75 mixture of the zinkiferous, or zinkiferous and plumbiferous, material and the reducing agent.

The reducing agent of the working charge 80 may be of any suitable kind, and while we now prefer to employ carbonaceous material as the reducing agent, it will be understood by those skilled in the art that reducing agents other than carbonaceous materials are available for the purposes of the 85 invention. One of the advantages of employing a briquetted reducing agent in any of the forms hereinbefore described is that it permits the use of carbonaceous materials 90 of cheaper grades and finer mesh, such as anthracite coal of finer mesh than No. 3 buckwheat, colliery washings, dust coal, coke breeze and the like.

The bed fuel briquets and the working 95 charge briquets may be prepared in any appropriate manner. We have found the procedure described in the aforementioned application of Frank G. Breyer, James A. Singmaster and Albert E. Hall, Serial No. 100 270,179, for preparing similar fuel and working charge briquets well adapted for the purposes of our present invention. This procedure involves generally the steps of mixing the material to be briquetted with a 105 suitable binder, such as concentrated waste sulfite liquor of 30° Baumé, molding the mixture into briquets of the desired size and shape, and drying or baking the briquets at a temperature of approximately 200° C., so 110 120 as to impart to them the desirable amount of resistance to crumbling and breaking so that they may be freely subjected to the rough handling incident to storing them, conveying them to the furnace, and incident 125 to charging them into the furnace either by hand or otherwise. In the case of the briquetted zinkiferous, or zinkiferous and plumbiferous, material, it is also desirable that the briquets possess such resistance to 130

crumbling and breaking as to substantially maintain their form during the entire furnacing operation, so that they are for the greater part discharged from the furnace 5 in substantially their original physical form.

The remaining novel features of the invention can be best explained by reference to the accompanying drawings, in which—

Figure 1 is a sectional elevation of an im-

- 10 proved furnace structure practically adapted for the practice of the invention; Fig. 2 is a side elevation of the same; Fig. 3 is a top plan of the furnace; Figs. 4, 5 and 6 are sectional views taken on the section lines 15 4—4, 5—5 and 6—6, respectively; Fig. 7 is a sectional view of the water-cooled leveler for the briqueted working charge, and Fig. 8 is a detail view of the perforated furnace hearth.

20 The furnace illustrated in the drawings has a movable or traveling hearth 10 in the form of a continuous belt or conveyer. The furnace hearth may advantageously be of the general design used in mechanical

25 stokers. As thus constructed, the hearth is made up of a plurality of metallic grate sections secured at their ends to sprocket chains 11. Each grate section is composed of a rigid frame piece having a dove-tailed web

30 on which are strung or keyed the relatively narrow members 12. The members 12 while mechanically contacting with one another permit the passage of the combustion supporting gas therebetween. The spaces between adjacent grate sections and between adjacent members 12 of each grate section provide perforations or small passages uniformly distributed over the entire area of the hearth.

35 The two sprocket chains 11 coöperate with and are driven by sprocket wheels 13 and 14 secured to shafts 15 and 16, respectively, at opposite ends of the furnace. The shafts 15 and 16 are connected through similar

40 worm reduction drives 17 and 18, beveled gears 19 and 20 and worm reduction drives 21 and 22, respectively, to a common shaft 23. The shaft 23 may be driven from any suitable power source, and to this end we

45 have represented a pulley 24, adapted to be operatively connected to the source of power, such, for example, as an electric motor. By this arrangement the shafts 15 and 16, at opposite ends of the furnace, are driven at the same speed, and the furnace hearth 10 is thereby positively driven by the coöperating sprocket wheels at each end of the furnace.

50 The furnace housing is constructed of fire brick in substantially the usual manner, with a casing of red brick on the outside. The brick work of the furnace structure, and in particular, the arches and skewbacks, are held in position by vertical buckstays 25 and 55 transverse tie-rods 26. The buckstays 25 are

preferably pivoted at their lower ends to anchor plates 27, preferably embedded in concrete. Relatively heavy coil springs 28 are associated with the tie-rods 26, for forcing coöperating pairs of buckstays on opposite sides of the furnace structure toward one another, thereby maintaining the buckstays firmly pressed against the skewback plates 29.

The skewback plates 29 are L-shaped, as 75 will be seen by reference to Figs. 4 and 6 of the drawings, and are arranged to support the skewbacks 30. The furnace arches are supported by the skewbacks 30 in the usual manner, as will be more particularly pointed 80 out hereinafter. It will be observed by reference to Figs. 4 and 6 of the drawings, that the buckstays 25 contact only with the skewback plates 29, and are thus separated by a small space from the side wall of the brick 85 work structure. By this arrangement the tie rods 26 and coöperating springs 28 serve to force each coöperating pair of buckstays firmly against the skewback plates 29, and thus any shrinkage in the brick work structure 90 of the furnace arch, as the furnace dries out, is taken care of and the danger of the arch falling in is practically eliminated. The pivot mounting of the buckstays 25 at their lower ends permits the necessary movement of the buckstays about this pivot to 95 compensate for shrinkage or expansion of the furnace arch.

The interior of the furnace housing is divided into a series of chambers by suspended arches. Thus, an ignition or fuel combustion chamber 31 is provided at the charging end of the furnace by the suspended arches 32 and 33. An ore combustion chamber 34 is provided between the suspended 100 arches 35 and 36. The arches 33 and 35 are suitably spaced in order to accommodate the charging devices for the briqueted working charge, as will be fully described hereinafter. The fume-emitting or oxid-making 105 chamber 79 of the furnace is located between the suspended arches 36 and 37.

Three off-takes 38, 39 and 40 are provided for conducting away from the fume-emitting zone the effluent produced therein as 110 the result of the operation. The off-takes 38, 39 and 40 may be connected to separate fume-collecting devices, or may communicate with a common flue and fume-collecting device. The ignition chamber 31 has an 115 off-take 41, and the ore combustion chamber 34 has an offtake 42. The gases passing through the offtakes 41 and 42 may be wasted or subjected to any proper treatment.

At the discharge end of the furnace a 120 chamber 43 is provided between the suspended arch 37 and the arch 37'. On one side of the chamber 43 there is an observation door 44, while on the other side there is a sliding door 45. These doors are provided as a 125

means of easy access to the rear sprockets 14. Observation doors 46 are provided at appropriate intervals on each side of the furnace opening directly into the combustion chambers or zones thereof.

The suspended arches 32, 33, 36 and 37 are held in position in substantially the same manner. Each of these arches is built of a plurality of rectangular fire brick.

10 Rods 47 are embedded in these rectangular fire bricks and passing upwardly through the furnace arch and roof are secured in place by being bolted to transverse beams 48. The sector-shaped spaces between the upper 15 surface of these rectangular fire bricks and the curved lower surface of the furnace arch are filled in with fire bricks so as to form the desired partition between the various chambers of the furnace.

20 The furnace arch or roof 49 is constructed of fire brick in the usual manner and is supported in position by the skewbacks 30, as will be well understood in the art. A cinder fill 50 may be placed on top of the 25 arch 49. Along each side wall of the furnace, just above the working surface of the traveling grate 10, carborundum bricks 51 are used to prevent fusion between the charge and the side walls of the furnace.

30 A hopper 52 is arranged at the front or charging end of the furnace for feeding the briqueted bed fuel on to the traveling grate. A gate or charge leveler 53 is associated with the hopper and is adapted to be raised or lowered by means of a wheel 54, and co-operating mechanism. By thus raising or lowering the gate 53, the depth of charge fed on to the traveling grate 10 may be regulated to the desired amount.

40 A hopper 55 is arranged to discharge into the space between the suspended arch 33 and the arch 35. A water-cooled gate or leveler 56 is arranged behind the hopper 55 for leveling the charge fed on to the traveling 45 grate by the hopper. The gate 56, as will be seen by reference to Fig. 7 of the drawings, comprises a hollow shell having transverse baffles 57 for imparting to the cooling medium flowing therethrough a circuitous path. This cooling medium, such, for example, as water, may be supplied to the interior of the hollow shell by an inlet pipe 58, and withdrawn by an outlet pipe 59. The 50 gate 56 is suspended from the top of the furnace structure by vertical rods 60 and may be vertically adjusted with respect to the moving grate by means of the nuts 61.

As hereinbefore explained, the drive for the traveling grate is connected so that the 60 grate is driven both from the front and rear through the main power shaft. The return grate is supported on riding bars 62 fastened to the side plates 63 of the furnace. The working floor of the furnace is supported on a suitable foundation 64, prefer-

ably elevated so as to facilitate the discharge of the exhaust material from the end of the furnace down an inclined chute 65 into cars or the like.

Above the return or lower portion of the 70 traveling grate 10, and out of contact therewith, is arranged a floor 66, which serves as the bottom wall of the air compartments beneath the upper or working surface of the traveling grate. Four air boxes 67 extend transversely of the furnace structure, at appropriate intervals between the front and rear thereof, and serve to admit the necessary blast of combustion supported gas beneath the perforated grate 10. The space 75 80 between adjacent air boxes 67 is divided into two compartments by means of the vertical partitions 68. By this arrangement it will be observed that eight air chambers or compartments are provided beneath the perforated traveling grate 10. Wear plates 67' and 68' are preferably mounted on the tops of the air boxes 67 and partitions 68, respectively, to serve as bearing plates for such portions of the traveling grate as contact therewith. The first air compartment at the front or charging end of the furnace is closed on the outside by a sheet metal wall 69, and a similar wall 70 closes the last air compartment at the rear or discharge 90 95 end of the furnace.

Each of the air boxes 67 extends exteriorly of the furnace at one side, as will be seen by reference to Figs. 2, 3 and 4 of the drawings. Each air box is connected exteriorly of the furnace by a vertical pipe 71 with the main air conduit 72. Each of the pipes 71 is provided with a slide valve 73, for regulating the air supply to its air box. Both of the transverse walls of each air 100 105 box 67 are provided with twyars or openings 74. A slide damper 75, terminating in a handle 76 exteriorly of the air box, is provided for each series of twyars 74. By moving the handles 76 in or out, the area 110 of the twyars or openings 74 can be adjusted, and in this manner the adjustment of the blast secured. It will be observed that while each air box serves to supply the combustion supporting gas to two air compartments, the amount of gas supplied to each compartment may be regulated by manipulation of the appropriate slide damper 75. 115

A trough 77 for water is preferably arranged in each of the air compartments, and a pipe 78 may connect with the troughs for conducting water thereto.

In practising the method of our present invention in the furnace illustrated in the accompanying drawings, the fuel briquets 125 are fed in at the front end of the grate through the hopper 52 and the thickness of the bed fuel is regulated by means of the gate 53, which, as hereinbefore explained, may be raised or lowered to any height de- 130

sired. From this point the fuel briquets travel into the fuel combustion chamber 31 and are there ignited by the high temperature maintained in this chamber. The 5 gases from the fuel combustion chamber are carried off through the stack 41.

At the rear of the fuel combustion chamber, just back of the suspended arch 33, the briquetted working charge is fed on to the 10 ignited fuel briquets through the hopper 55. The depth of the briquetted working charge is regulated by the gate 56, which may be set at any desired height. As previously 15 explained, this gate is cooled by means of circulating water. The briquetted working charge thus spread on the ignited fuel briquets is advanced into what we have called the ore combustion chamber 34, in which the charge is brought up to the reducing 20 temperature. The stack 42 is provided so that, if desirable, the effluent made in this chamber may be recovered separately from that produced in the main oxid-making chamber 79.

25 The briquetted charge now passes under the suspended arch 36 into the main effluent or oxid-making chamber 79, in which the active reduction of the charge takes place. The blow or blast in this chamber is so regulated that complete reduction takes place 30 by the time the charge has traveled to the rear of the chamber. From the oxid-making chamber the three off-takes 38, 39 and 40 conduct the effluent to the oxid drum, as 35 will be well understood in the art. Each of the off-takes 42, 38, 39 and 40, is provided with a slide damper 42', 38', 39' and 40', respectively, for regulating the flow of the effluent so as to help control the temperature 40 at all points of the chamber 79. A trailing door or gate 80 is operatively mounted on the suspended arch 37 for preventing the passage underneath the arch and into the chamber 79 of currents or drafts of air.

45 From the main oxid-making chamber 79, the worked off briquets pass underneath the suspended arch 37 into the rear chamber 43. This chamber is also provided with a stack 82, for balancing the draft between 50 the rear chamber and the oxid making chamber. As the grate sections pass over the rear sprockets 14, the worked-off charge, consisting of a light coal clinker and worked-off briquets, is discharged onto the 55 chute 65 and thence into the receiving hoppers (not shown). A pendant door or gate 81 is pivoted to the arch 37' and serves to maintain the residue-discharge opening of the chamber 43 normally closed. When a 60 certain amount of residue banks up against this door 81 it swings open to permit the discharge of the residue down the chute 65.

The traveling furnace hearth moves at a very slow speed, a few feet per hour. The 65 speed of the hearth will be determined by the

dimensions of the fume-emitting zone, the character and quantity of zinkiferous material charged and other considerations, which will be understood by those skilled in the art. We have found a temperature of approximately 1100 to 1250° C. well suited for the fume-emitting or oxid-making chamber or zone, when using the well known Franklin furnace zinc oxid ores, and at this temperature the briquetted working charge can ordinarily be satisfactorily worked-off or depleted of its zinkiferous content in from two and one-half to three and one-half hours, when operating with a furnace whose oxid-making chamber 79 is about eighteen feet in 80 length and with a grate speed of about seven feet per hour.

In the customary commercial practice of the Wetherill process, the total carbonaceous material in the entire charge, including the 85 bed fuel and the working charge mixture, is several times greater than the theoretical amount required to reduce the zinkiferous material in the charge. It has heretofore been the general practice to place the greater 90 proportion of the total carbonaceous material of the charge in the working charge mixture. For example, when operating with the well known Franklin furnace zinc oxid ores, it is customary to place from about 15 to 25 95 per cent. of the total carbonaceous material of the entire charge in the bed fuel, while the remaining 85 to 75 per cent. of the total carbonaceous material is mixed with the ore to form the working charge. In general 100 terms, the layer of bed fuel is approximately one inch in depth or thickness, while the working charge mixture is spread over the ignited bed fuel in a layer from about five to seven inches in depth or thickness.

A very decided improvement in the efficiency of the Wetherill process can be secured by placing the greater proportion of the total fuel of the charge in the form of briquets in the bed fuel, rather than in the 110 working charge as has heretofore been customary. This improvement in the heretofore customary practice of the Wetherill process is described and claimed in an application for Letters Patent of the United 115 States of Frank G. Breyer, Albert E. Hall and George R. Waltz, Serial No. 310,439, filed July 12, 1919. When a very considerable proportion of the carbonaceous or other combustible material of the entire charge is 120 thus withdrawn from the working charge and placed in the bed fuel in the form of briquets, the residual charge consists of a relatively thin clinkered ash, resulting from the combustion of the bed fuel briquets, and the worked-off metalliferous material. When the zinkiferous material has been briquetted and spread on the ignited bed fuel briquets, the worked-off ore briquets are discharged in substantially their original physical form,

70

75

80

85

90

95

100

105

110

115

120

125

130

so that the worked-off briquets may be readily separated from the clinkered ash of the bed fuel briquets. Furthermore, in view of the fact that the working charge briquets 5 contain only a relatively small amount of the total carbonaceous material of the charge, the resulting amount of ash in the worked-off ore briquets is relatively small, and such worked-off briquets may on this account be 10 very advantageously employed in subsequent smelting operations for the recovery therefrom of further metallic values, as will be more fully described hereinafter. Accordingly, in view of the attendant advantages, it 15 is our preferred practice in carrying out the present invention to place the greater part of the total carbonaceous or combustible material of the entire charge in the bed fuel briquets, and we have secured excellent re- 20 sults by placing from about 75 to about 85% of the total combustible material of the entire charge in the bed fuel briquets. 75

As a typical instance of the practice of the invention, we will now describe a particular operation in which both fuel briquets and a briquetted working charge were used. Eighty-five (85) per cent. of the total coal of the entire charge was carried in the bed fuel briquets, leaving fifteen (15) per cent. 30 of the total coal for mixture with the zinkiferous material in the working charge. The fuel briquets were made up of dust coal with three (3) per cent. concentrated waste sulfite liquor binder. The briquetted working charge consisted of a mixture of ninety (90) per cent. Franklin furnace zinc oxid ore and ten (10) per cent. dust coal, to which three (3) per cent. waste sulfite liquor was 35 added as a binder. Both the ore and fuel briquets were of the rounded pillow block type. 40

The levelers or gates 53 and 56 of the accompanying drawings were set to deliver a layer of bed fuel six inches deep and a three 45 inch layer of the briquetted working charge.

In the foregoing operation, we secured very satisfactory results by holding the fuel ignition chamber 31 at the minimum temperature for uniform ignition, that is, from 50 about 800° to 950°C.; the ore ignition chamber 34 at a temperature where a light zinc flame is visible, for example, from 1000° to 1050° C., and the oxid-making chamber 79, at a uniform temperature of from 1100° 55 to 1250° C., since at this temperature reduction is active, and with the usual working mixtures only incipient fusion of the briquetted working charge takes place.

No bars or rakes need be used, nor need 60 the charge be disturbed in any manner in practising the method of our present invention. The only labor necessary consists in feeding the briquets to the furnace and carting away the clinker and worked-off 65 briquets discharged into the hoppers or cars

provided therefor. There is, furthermore, no blow-hole trouble, and no sticking of the charge to the side walls and no loss of blow at the side walls. The briquets feed uniformly and the ignition of both fuel and 70 working charge briquets is very uniform. The clinker, consisting of a relatively thin layer of coal ash and burned-out briquets, discharges readily and no labor is attendant upon the discharging operation. 75

The oxid made in accordance with our invention is decidedly superior to that made from charges of the same ore on the customary oxid furnace blocks. It is particularly free from any grit or specks and very 80 bright. The recoveries of zinc from the working charge are remarkably high, and we have found by the practice of our invention, that it is possible to secure recoveries better than ninety per cent., as indicated 85 by the clinker analysis.

When, as in the preferred embodiment of the invention, the zinkiferous, or zinkiferous and plumbiferous, material of the working charge is supplied to the furnace 90 hearth in the form of briquets, the worked-off ore briquets retain for the most part their original shape with only incipient fusion. Some of the working charge briquets will almost inevitably become broken or crushed 95 in the preliminary handling and furnacing operation, but these briquets for the greater part retain their original physical form. After the furnacing operation, these briquets are remarkably hard and almost coke-like 100 in their physical characteristics, and are readily separated from the clinkered coal ash of the bed fuel briquets.

This capability of readily separating the worked-off ore briquets from the ash of the 105 fuel briquets is of especial advantage when the worked-off metalliferous briquets are to be subjected to further treatment for the recovery of valuable metals not volatilizable by the Wetherill process. Where the work- 110

ing charge briquets consist of a mixture of zinkiferous or zinkiferous and plumbiferous material and carbonaceous reducing agent, the worked-off briquets will contain, in addition to the worked-off zinkiferous, or 115 zinkiferous and plumbiferous material, the ash from the consumed carbonaceous reducing agent as well as the unconsumed portion of the reducing agent. The ash is composed principally of silica and alumina, 120 and is generally objectionable in any subsequent treatment of the worked-off ore briquets. Thus, for example, in those instances in which the worked-off ore briquets are smelted in a blast furnace for the production of spiegeleisen a certain amount of 125 fluxing agents is necessary for slagging off the ash present in the worked-off ore briquets, and when this amount of ash is relatively large an objectionably large amount 130

of fluxing agent is required, with the resultant production of an objectionably large amount of slag. By placing approximately 85% of the total carbonaceous material of 5 the entire charge in the bed fuel briquets, the main bulk, for example, around eighty-five (85) per cent., of the ash of the total carbonaceous material of the charge is in the clinker resulting from the combustion 10 of the bed fuel briquets, and the worked-off ore briquets are consequently contaminated with only a relatively small amount of ash. On account of this relatively slight ash contamination of the worked-off ore briquets, 15 as well as on account of their physical properties, these briquets are peculiarly well adapted for subsequent treatment in blast furnaces. In addition to retaining their original form, these briquets are moreover 20 of a porous character, due to the removal of the zinc, or zinc and lead, therefrom, and this porous property of the worked-off briquets is also of advantage in their subsequent treatment.

25. A very accurate and uniform control of the temperature throughout the entire furnace, and hence during the entire furnacing operation of the charge, is secured by the practice of the invention. Thus, the temperature 30 of the various chambers or zones of the furnace can be accurately regulated and controlled by appropriately adjusting the slide dampers 73 of the various air compartments, and the desired operating temperatures 35 are easily maintained throughout the entire furnace. This uniformity of the temperature conditions is attended by practically uniform working conditions of the desired character throughout the furnace, and 40 results in the production of a uniform product of improved quality as well as in increased output. The furnacing operation is substantially automatic, and requires only casual attention, thereby effecting a great 45 saving in labor over that required in the operation of the present day types of oxid furnaces. The combustion of the bed fuel is substantially complete, so that practically the full caloric value of the fuel is effectively 50 utilized, thereby enabling a saving in the amount of fuel required as compared with that necessary in working with the heretofore customary types of oxid furnaces. The worked-off briquets are, in our preferred 55 practice, only slightly contaminated with ash and the like, and on this account, as well as on account of their physical form and properties these worked-off briquets are well adapted for subsequent smelting operations.

60. We claim:

1. The process of producing zinc oxid or leaded zinc oxid which comprises advancing through a suitable combustion zone a working charge containing a briqueted mixture 65 of zinkiferous or zinkiferous and plumbifer-

ous material and a reducing agent spread on an ignited layer of bed fuel in the form of briquets and simultaneously passing a combustion supporting gas into the charge, and removing the resulting effluent; substantially as described. 70

2. The process of producing zinc oxid or leaded zinc oxid which comprises advancing through a suitable combustion zone a working charge containing a mixture of briqueted 75 zinkiferous or zinkiferous and plumbiferous material and a reducing agent spread on an ignited layer of bed fuel in the form of briquets and simultaneously passing a combustion supporting gas into the charge, and 80 removing the resulting effluent; substantially as described.

3. The process of producing zinc oxid or leaded zinc oxid which comprises advancing through a suitable combustion zone a working charge containing briqueted zinkiferous or zinkiferous and plumbiferous material spread on an ignited layer of bed fuel in the form of briquets and simultaneously passing a combustion supporting gas into the 85 charge, and removing the resulting effluent; substantially as described.

4. The process of producing zinc oxid or leaded zinc oxid which comprises advancing through a suitable combustion zone a working charge containing a mixture of zinkiferous or zinkiferous and plumbiferous material and a briqueted reducing agent spread on an ignited layer of bed fuel in the form of briquets and simultaneously passing a combustion supporting gas into the charge, and 90 removing the resulting effluent; substantially as described. 95

5. The process of producing zinc oxid or leaded zinc oxid which comprises advancing through a suitable combustion zone a working charge containing a mixture of zinkiferous or zinkiferous and plumbiferous material spread on an ignited layer of bed fuel in the form of briquets 100 and simultaneously passing a combustion supporting gas into the charge, and removing the resulting effluent; substantially as described. 105

6. The process of producing zinc oxid or leaded zinc oxid which comprises advancing through a suitable combustion zone a working charge containing zinkiferous or zinkiferous and plumbiferous material spread on an ignited layer of bed fuel in the form of briquets 110 and simultaneously passing a combustion supporting gas into the charge, and removing the resulting effluent; substantially as described. 115

7. The process of producing zinc oxid or leaded zinc oxid which comprises advancing through a suitable combustion zone a working charge containing a briqueted mixture of zinkiferous or zinkiferous and plumbiferous material and a reducing agent spread 120

125

on an ignited layer of bed fuel and simultaneously passing a combustion supporting gas into the charge, and removing the resulting effluent; substantially as described.

5 8. The process of producing zinc oxide or leaded zinc oxide which comprises advancing through a suitable combustion zone a working charge containing a mixture of briqueted zinkiferous or zinkiferous and plumbiferous

10 material and a reducing agent spread on an ignited layer of bed fuel and simultaneously passing a combustion supporting gas into the charge, and removing the resulting effluent; substantially as described.

15 9. The process of producing zinc oxid or leaded zinc oxid which comprises advancing through a suitable combustion zone a working charge containing briqueted zinkiferous or zinkiferous and plumbiferous material

20 10. The process of producing zinc oxid or leaded zinc oxid which comprises spreading on an ignited layer of bed fuel and simultaneously passing a combustion supporting gas into the charge, and removing the resulting effluent; substantially as described.

25 10. The process of producing zinc oxid or  
lead zinc oxid which comprises depositing  
upon a perforated hearth a layer of bed fuel  
in the form of briquets, igniting said layer  
of briquets, spreading thereon a working  
30 charge containing a briqueted mixture of  
zinkiferous or zinkiferous and plumbiferous  
material and a reducing agent, advancing  
said hearth and the charge supported there-  
on through a combustion zone and simul-  
35 taneously passing a combustion supporting  
gas into the charge, and removing the re-  
sulting effluent; substantially as described.

11. The process of producing zinc oxide or leaded zinc oxide which comprises depositing upon a perforated hearth a layer of bed fuel in the form of briquets, igniting said layer of briquets, spreading thereon a working charge containing a mixture of briquetted zinkiferous or zinkiferous and plumbiferous material and a reducing agent, advancing said hearth and the charge supported thereon through a combustion zone and simultaneously passing a combustion supporting gas into the charge, and removing the resulting effluent; substantially as described.

12. The process of producing zinc oxid or leaded zinc oxid which comprises depositing upon a perforated hearth a layer of bed fuel in the form of briquets, igniting said layer of briquets, spreading thereon a working charge containing briqueted zinkiferous or zinkiferous and plumbiferous material advancing said hearth and the charge supported thereon through a combustion zone and simultaneously passing a combustion supporting gas into the charge, and removing the resulting effluent; substantially as described.

### 65 13: The process of producing zinc oxid or

lead zinc oxid which comprises depositing upon a perforated hearth a layer of bed fuel in the form of briquets, igniting said layer of briquets, spreading thereon a working charge containing a mixture of zinkiferous or zinkiferous and plumbiferous material and a briquetted reducing agent, advancing said hearth and the charge supported thereon through a combustion zone and simultaneously passing a combustion supporting gas into the charge, and removing the resulting effluent; substantially as described.

14. The process of producing zinc oxid or leaded zinc oxid which comprises depositing upon a perforated hearth a layer of bed fuel in the form of briquets, igniting said layer of briquets, spreading thereon a working charge containing a mixture of zinkiferous or zinkiferous and plumbiferous material and a reducing agent, advancing said hearth and the charge supported thereon through a combustion zone and simultaneously passing a combustion supporting gas into the charge, and removing the resulting effluent; substantially as described. 80 85 90

15. The process of producing zinc oxide or leaded zinc oxide which comprises depositing upon a perforated hearth a layer of bed fuel in the form of briquets, igniting said layer 95 of briquets, spreading thereon a working charge containing zinkiferous or zinkiferous and plumbiferous material, advancing said hearth and the charge supported thereon through a combustion zone and simultaneously passing a combustion supporting gas into the charge, and removing the resulting effluent; substantially as described. 100

16. The process of producing zinc oxid or leaded zinc oxid which comprises depositing upon a perforated hearth a layer of bed fuel, igniting said layer of bed fuel, spreading thereon a working charge containing a briqueted mixture of zinkiferous or zinkiferous and plumbiferous material and a reducing agent, advancing said hearth and the charge supported thereon through a combustion zone and simultaneously passing a combustion supporting gas into the charge, and removing the resulting effluent; substantially as described. 110 115

17. The process of producing zinc oxide or leaded zinc oxide which comprises depositing upon a perforated hearth a layer of bed fuel, igniting said layer of fuel, spreading thereon a working charge containing a mixture of briqueted zinkiferous or zinkiferous and plumbiferous material and a reducing agent, advancing said hearth and the charge supported thereon through a combustion zone and simultaneously passing a combustion supporting gas into the charge, and removing the resulting effluent; substantially as described. 120 125

### 18. The process of producing zinc oxide 130

or leaded zinc oxid which comprises depositing upon a perforated hearth a layer of bed fuel, igniting said layer of bed fuel, spreading thereon a working charge containing briqueted zinkiferous or zinkiferous and plumbiferous material, advancing said hearth and the charge supported thereon through a combustion zone and simultaneously passing a combustion supporting gas into the charge, and removing the resulting effluent; substantially as described.

19. The process of producing zinc oxid or leaded zinc oxid which comprises depositing upon a furnace hearth a layer of bed fuel containing the greater part of the total combustible material of the entire charge in the form of briquets, igniting said layer of bed fuel briquets, spreading thereon a working charge containing a briqueted mixture of zinkiferous or zinkiferous and plumbiferous material and a reducing agent, advancing said hearth and the charge supported thereon through a combustion zone and simultaneously passing a combustion supporting gas into the charge, and removing the resulting effluent; substantially as described.

20. The process of producing zinc oxid or leaded zinc oxid which comprises depositing upon a furnace hearth a layer of bed fuel containing the greater part of the total combustible material of the entire charge in the form of briquets, igniting said layer of bed fuel briquets, spreading thereon a working charge containing a mixture of briqueted zinkiferous or zinkiferous and plumbiferous material and a reducing agent, advancing said hearth and the charge supported thereon through a combustion zone and simultaneously passing a combustion supporting gas into the charge, and removing the resulting effluent; substantially as described.

21. The process of producing zinc oxid or leaded zinc oxid which comprises depositing upon a furnace hearth a layer of bed fuel containing the greater part of the total combustible material of the entire charge in the form of briquets, igniting said layer of bed fuel briquets, spreading thereon a working charge containing briqueted zinkiferous or zinkiferous and plumbiferous material, advancing said hearth and the charge supported thereon through a combustion zone and simultaneously passing a combustion supporting gas into the charge, and removing the resulting effluent; substantially as described.

22. The process of producing zinc oxid or leaded zinc oxid which comprises deposit-

ing upon a furnace hearth a layer of bed fuel containing the greater part of the total combustible material of the entire charge in the form of briquets, igniting said layer of bed fuel briquets, spreading thereon a working charge containing a mixture of zinkiferous or zinkiferous and plumbiferous material and a briqueted reducing agent, advancing said hearth and the charge supported thereon through a combustion zone and simultaneously passing a combustion supporting gas into the charge, and removing the resulting effluent, substantially as described.

23. The process of producing zinc oxid or leaded zinc oxid which comprises depositing upon a furnace hearth a layer of bed fuel containing the greater part of the total combustible material of the entire charge in the form of briquets, igniting said layer of bed fuel briquets, spreading thereon a working charge mixture containing sinkiferous or zinkiferous and plumbiferous material and a reducing agent, advancing said hearth and the charge supported thereon through a combustion zone and simultaneously passing a combustion supporting gas into the charge, and removing the resulting effluent, substantially as described.

24. The process of producing zinc oxid or leaded zinc oxid which comprises depositing upon a furnace hearth a layer of bed fuel containing the greater part of the total combustible material of the entire charge in the form of briquets, igniting said layer of bed fuel briquets, spreading thereon a working charge containing zinkiferous or zinkiferous and plumbiferous material, advancing said hearth and the charge supported thereon through a combustion zone and simultaneously passing a combustion supporting gas into the charge, and removing the resulting effluent, substantially as described.

25. In a process for producing zinc oxid or leaded zinc oxid involving the blowing of air into a continuously advancing bed containing a metal-bearing material and combustible material under conditions which will leave the worked-off charge as a clinker and which will produce a volatile fume, the step of supplying at least part of the charge in the form of briquets; substantially as described.

In testimony whereof we affix our signatures.

JAMES A. SINGMASTER.  
FRANK G. BREYER.  
EARL H. BUNCE.